

May 7, 1940.

J. R. ALBURGER

2,199,902

PHOTOGRAPH

Filed April 12, 1938

*Fig. 1.*



*Fig. 2.*



Inventor

James R. Alburger

By

*J. J. Jaff*

Attorney

## UNITED STATES PATENT OFFICE

2,199,902

## PHOTOGRAPH

James R. Alburger, Merion, Pa., assignor to Radio Corporation of America, a corporation of Delaware

Application April 12, 1938, Serial No. 201,507

2 Claims. (Cl. 95—88)

This invention relates to an improved photographic image, and particularly to an improved photographic image produced in gelatine sensitized by a silver salt.

5 In my application Serial No. 196,366, filed March 17, 1938 (RCV Docket 5657), entitled "Photographic developer," are described certain improvements in the composition of photographic developers. The present application is related 10 thereto in that it pertains to a photographic image or photograph produced by the use of the aforesaid and other developers.

My improved photograph has the characteristic that the image is formed not only from 15 reduced silver grains, but also from a mordant deposited in the gelatine and which may in itself be colored, or may be colorless and impregnated with a dye, or both.

In the production of my improved photograph, 20 I use a developer such as that referred to in my aforesaid application, which maintains a mordant material in solution and which, during the action of the developer, deposits the said material around and between the silver grains in proportion to the amount of developing action occurring.

One object of my invention is to provide an improved photograph.

Another object of my invention is to provide 30 a photograph having improved contrast.

Another object of my invention is to provide a photograph having greater density than heretofore possible.

Another object of my invention is to provide 35 an improved photograph capable of being tinted.

Another object of my invention is to provide a photograph reducing the effect of graininess.

Another object of my invention is to provide a photographic image which is capable of being converted into a dye image.

40 Another object of my invention is to provide a photographic dye image coincident with a photographic silver image.

Other and incidental objects of my invention 45 will be apparent to those skilled in the art from a reading of the following specification and an inspection of the accompanying drawing, in which

Figure 1 is a greatly enlarged view of a photograph, a photograph of a sound record being chosen for purposes of illustration, and

Figure 2 is a sectional view taken along the line 2—2 of Fig. 1.

As shown in the drawing, a base 1 of any of 50 the usual materials such as glass, Celluloid, pa-

per or the like, is provided. On this is superposed the usual emulsion layer 2, which may be of any convenient type such, for example, as is used on commercial motion picture film, in which case the base 1 would be of Celluloid or cellulose acetate. The emulsion 2 is, prior to exposure, replete with grains of silver salt, such as silver bromide, silver iodide, silver chloride, or a combination of two or more of these substances.

5 Exposure is accomplished in the usual fashion, and the film is then developed in a developer having in solution a mordanting agent such as aluminum hydroxide. As an example of one developer suitable for the purpose, the following may be used:

|                                                             |       |       |
|-------------------------------------------------------------|-------|-------|
| Hydroquinone (para-dihydroxybenzene) ---                    | grams | 15    |
| Na <sub>2</sub> SO <sub>3</sub> ---                         | do    | 17    |
| KAl(SO <sub>4</sub> ) <sub>2</sub> · 12H <sub>2</sub> O --- | do    | 38    |
| NaOH ---                                                    | do    | 30 20 |
| KBr ---                                                     | do    | 10    |
| Water to make                                               | ccs.  | 1000  |

An alternative formula is:

|                                                             |       |         |
|-------------------------------------------------------------|-------|---------|
| Na <sub>2</sub> SO <sub>3</sub> ---                         | grams | 50 25   |
| Mono-methyl carboxyl paramino hydroxybenzene (Glycin) ---   | grams | 20      |
| NaOH ---                                                    | do    | 25      |
| KAl(SO <sub>4</sub> ) <sub>2</sub> · 12H <sub>2</sub> O --- | do    | 30      |
| Water to make                                               | ccs.  | 1000 30 |

The invention is by no means limited to the use of the foregoing two formulas, but my improved photograph may be obtained by the use of any developer containing an appropriate mordanting material in solution. For example, I 35 have found that a developer using any of the conventional benzene or naphthalene derivative developing agents, and having either aluminum alum or chrome alum maintained in solution by sufficient alkali to redissolve the precipitate tending to be first formed on the addition of the alum, will accomplish my purpose.

Upon development of the exposed emulsion, 45 the grains of silver salts, such as indicated at 3, are reduced to metallic silver in the usual discrete form. During such reduction, however, the bromine, iodine, or chlorine which is liberated from the silver salts reacts with the alkali of the developer to produce the corresponding sodium salt at the point of development. This reaction drops the alum out of solution at the point of development, leaving aluminum hydroxide, chromium hydroxide or the like deposited around and between the developed silver grains, and since 50 55

the amount of sodium hydroxide changing into a salt is dependent upon the amount of silver changing from the halide to metallic silver, the amount of aluminum or chromium hydroxide deposited at that point corresponds to the amount of silver reduced. As is well known, these hydroxides are not soluble in water and are very effective mordanting agents for acid dyes. The deposited hydroxide is indicated in the drawing 10 at 4.

If desired, this hydroxide may be treated with any appropriate dye such as any of those which are used commercially in conjunction with aluminum hydroxide as a mordant, these types being generally referred to as acid dyes. The chromium salts, having some color themselves, add 15 to the density of the silver image without the addition of dye.

If desired, the appropriate dye may be added 20 directly to the developer in appropriate amount, subject only to the limitation that, in this case, a dye must be chosen which does not react with the developing agent itself, and which of the

aforesaid dyes can be used depends upon the specific developing agent chosen, and vice versa.

If desired, either before or after dyeing the deposited silver may be removed by an appropriate silver solvent such, for example, as the well known "Farmer's reducer," composed of a solution of sodium hyposulphite and potassium ferricyanide. For the purpose of removing the silver, such an agent as the usual potassium bichromate-sulphuric acid solution should be 10 avoided, as the sulphuric acid has a tendency to dissolve the mordant.

Having described my invention, I claim:

1. A photograph including a reduced silver image and a coincident aluminum hydroxide 15 mordant image.

2. A photograph comprising a base, a gelatine emulsion on said base, a reduced silver image in said emulsion, and a deposited aluminum hydroxide mordant image coincident with said 20 silver image.

JAMES R. ALBURGER.